# EUROPEAN PATENT SPECIFICATION

(11) **EP 3 003 607 B1**
(45) Date of publication and mention of the grant of the patent: **27.05.2020**
(21) Application number: 14806817.4
(22) Date of filing: 28.05.2014
(51) Int. Cl.: B22F 1/00, B22F 3/14, B22F 3/22

(54) **SLIP AND PRESSURE CASTING OF REFRACTORY METAL BODIES**
GLEIT- UND DRUCKGIESSEN VON FEUERFESTEN METALLKÖRPERN
COULAGE EN BARBOTINE ET SOUS PRESSION DE CORPS EN MÉTAL RÉFRACTAIRE

(30) Priority: 04.06.2013 US 201361830892 P
(43) Date of publication of application: 13.04.2016
(73) Proprietor: H. C. Starck Inc, Newton, MA 02461 (US)
(72) Inventor: STAWOVY, Michael, T., Cleveland Heights, OH 44118 (US); WINNICKA, Maria, Bozena, Euclid, OH 44123 (US)
(74) Representative: Maiwald Patent- und Rechtsanwaltsgesellschaft mbH
(86) International application number: PCT/US2014/039708
(87) International publication number: WO 2014/197246

(56) References cited:
- EP-A1- 2 559 678
- EP-A2- 1 077 099
- EP-B1- 0 905 107
- JP-A- H04 124 204
- JP-A- 2000 272 951
- US-A- 3 578 478
- US-A- 3 917 778
- US-A1- 2009 123 690

## Description

### Related Application

This application claims the benefit of and priority to U.S. Provisional Patent Application No. 61/830,892, filed June 4, 2013.

### Technical Field

In various embodiments, the present invention relates to slip casting with or without applied pressure, in particular to such slip or pressure casting of metal bodies.

### Background

Powder metallurgy techniques have been utilized in the fabrication of various types of finished metallic parts. For example, a flexible bag may be filled with metal powder and placed in a mold that approximates the final pressed shape and dimensions of the part. The bag and mold are sealed, and cold isostatic pressing is utilized to form a pressed "green body" of the metal powder. The green body may then be sintered in order to increase its density and subsequently machined to its final desired dimensions. While such powder metallurgy techniques are useful for particular applications, their utility is limited when the final parts have more complicated shapes. The more complicated the shape, the more excess powder must be placed in the bag and mold in order to prevent cracking during pressing. Thus, the ratio of the weight of the sintered part to the new weight of the part in its final machined form may exceed 4:1, resulting in high machining, materials, and labor costs. Moreover, parts fabricated with such powder metallurgy techniques rarely achieve final sintered densities that exceed 94% of their theoretical densities. Such parts may also have disadvantageously large grain sizes, e.g., greater than 40 microns.

Another powder metallurgy technique utilized for the production of complex shapes is slip casting, in which a "slip," i.e., a suspension of fine metal powder in water, dispersing agents (for the stabilization of the powder against colloidal forces), one or more solvents (for control of slip viscosity and facilitating casting), and a binder for strengthening the cast shape are placed in a mold, the liquids are drawn away, and the resulting green body is sintered for densification and strength. Unfortunately, slip casting typically requires the use of a deflocculant or suspension aid to prevent the settling and agglomeration of the powder and to maintain a desirable slip viscosity. Such deflocculants include, e.g., alcohols, other organic liquids, or alginates (i.e., ammonium and sodium salts of alginic acids). The use of such additives increases the cost, complexity, environmental impact and materials-handling requirements for a slip-casting process. Document US3578478A describes a method of producing a shaped part in which a tungsten powder having discrete particle sizes is suspended in water for slip casting without separation of the particles.

In view of the foregoing, there is a need for simplified powder metallurgy-based techniques for the fabrication of complex metal parts that do not utilize exotic additives and that enable high part densities and small final grain sizes.

### Summary

In accordance with various embodiments of the present invention, metal parts (or "bodies") are produced utilizing slip or pressure casting of metal powders having specific powder-size distributions that obviate the need for the use of added organic or inorganic suspension aids during casting. The metal powders are suspended in a liquid that includes or consists essentially of water, e.g., deionized (DI) water, and poured into a mold for casting. As mentioned above, the liquid does not include any flocculating or deflocculating additives. In addition, preferred embodiments utilize powders that consist essentially only of one or more metals and do not contain solid or powder agents such as binders or plasticizers. The mold is porous (and may include or consist essentially of, e.g., gypsum), and the liquid in which the powder is suspended is drawn into the mold via capillary action. The resulting green body is sintered to increase its density and final machining (if desired and/or necessary) is performed to shape the final part. The metal powder may include or consist essentially of, e.g., one or more refractory metals. For example, the metal powder may include or consist essentially of tungsten (W), tantalum (Ta), niobium (Nb), zirconium (Zr), molybdenum (Mo), and/or titanium (Ti).

In general, the slip does not exhibit dilatant or thixotropic flow, for example, when the slip is being poured into the mold; rather, the viscosity of the slip is preferably approximately constant as a function of the shear rate (i.e., with changes in shear rate) applied to the slip. Moreover, in preferred embodiments of the invention the slip and/or mold is not agitated (e.g., stirred, shaken, rotated, and/or vibrated) to promote mixing or settling of the metal powder within the slip; rather, the engineered particle size distribution of the powder particles within the slip provides resistance to powder settling within the slip before and during casting (i.e., the slip is colloidally stable rather than, e.g., colloidally unstable or even metastable, in preferred embodiments) while also facilitating low-resistance pourability of the slip itself in the absence of agitation. Similarly, in preferred embodiments of the present invention no electrical voltage or current is applied to the mold or slip during the casting process to influence settling behavior. In addition, the green bodies and molded parts (before and after sintering) are generally not functionally or mechanically graded, i.e., the parts exhibit few if any gradients in composition, microstructure, mechanical properties, porosity, residual stress, grain size, particle size, etc. Instead, the mechanical and functional properties of bodies and parts fabricated in accordance with embodiments of the present invention (e.g., grain size of unsintered or sintered parts, and/or powder particle size of slips and/or green bodies) are substantially homogeneous in various (or even all) directions. Furthermore, embodiments of the invention feature slips that are substantially free of acidic or basic pH-modifying agents; such agents may have deleterious effects (e.g., corrosion and/or chemical reaction) on the metal powder particles utilized in preferred embodiments and are generally not necessary for engineering colloidal stability of slips described herein.

As utilized herein, the terms "body," "part," and "article" refer to bulk three-dimensional objects (as opposed to mere grains of powder) with shapes as simple as a slab but also more complex shapes such as crucibles and other volumes having convexity and/or concavity. For complex shapes, the final shape (not considering any process-related shrinkage) is typically formed by casting (as opposed to bulk compression) and sintering, which may be followed by machining.

In an aspect, embodiments of the invention feature a method of producing a shaped part. A powder is suspended in a liquid consisting essentially of water, thereby forming a slip. The powder has a particle-size distribution d10 between 0.15 micron and 0.5 micron, d50 between 0.6 micron and 1 micron, and d90 between 2.4 microns and 3 microns, where a particle-size distribution dX of Y denotes that X% of particles have a size less than Y. The slip is introduced into a mold having a shape approximately equal to a desired shape of the shaped part. The particle-size distribution of the powder (i) substantially prevents separation of the powder from the liquid by agglomeration and/or sedimentation and (ii) maintains a substantially homogeneous distribution of powder particles within the liquid. Thereafter, at least a portion of the liquid drains out of the slip to produce a green body comprising or consisting essentially of the powder, and the green body is sintered to produce the shaped part.

Embodiments of the invention may include one or more of the following in any of a variety of different combinations. The particle-size distribution of the powder may be d10 of approximately 0.3 micron, d50 of approximately 0.8 micron, and d90 of approximately 2.7 microns. After sintering, the shaped part may have a density between approximately 95% and approximately 99% of theoretical density, or even between 97% and 99% of theoretical density. After sintering, the shaped part may have a grain size (e.g., average grain size) between approximately 10 microns and approximately 20 microns. The powder includes or consists essentially of one or more refractory metals. The powder may include or consist essentially of tungsten, tantalum, niobium, zirconium, molybdenum, and/or titanium. The green body may be sintered in hydrogen. The green body may be sintered at a temperature between approximately 3000 °F (1649°C) and approximately 5000 °F (2760°C).

The powder may be produced by providing an initial powder having a particle-size distribution d10 of approximately 0.42 micron, d50 of approximately 1.8 micron, and d90 of approximately 3.8 microns, deagglomerating a portion of the initial powder, and blending the deagglomerated portion of the initial powder with a second portion of the initial powder. The portion of the initial powder may be deagglomerated by ball milling. The density of the green body may be between approximately 30% and approximately 40% of theoretical density. The liquid may consist essentially of deionized water. The mold may be porous. Substantially all of the liquid from the slip may drain into the mold to form the green body. Neither the slip nor the mold may be agitated (e.g., shaken, stirred, vibrated, and/or rotated) after the slip is introduced into the mold and before the green body is produced. A super-atmospheric pressure (which may be hydrostatic) is applied to the mold and/or to the slip during and/or after introducing the slip into the mold. The powder may be substantially homogeneously distributed within the green body (i.e., there may be no noticeable gradients or bands in particle or grain size formed within the green body). The mold may contain substantially only the slip. The shaped part may be machined to a desired size and/or shape.

Additionally, outside the scope of the invention a method of producing a shaped part is provided. A powder is suspended in water without flocculating or deflocculating additives, thereby forming a slip. The slip is introduced into a mold having a shape approximately complementary to (i.e., enclosing a space for introduction of slip therewithin approximately equal to) a desired shape of the shaped part substantially without separation of the powder from the water (and/or settling or sedimentation of the powder within the water) thereduring. Thereafter, at least a portion of the liquid is allowed to drain out of the slip to produce a green body including or consisting essentially of the powder, and the green body is sintered to produce the shaped part.

Embodiments of the invention may include one or more of the following in any of a variety of different combinations. The powder may have a particle-size distribution (i) substantially preventing separation of the powder from the water by at least one of agglomeration or sedimentation and (ii) maintaining a substantially homogeneous distribution of powder particles within the liquid. The particle-size distribution may be d10 between 0.15 micron and 0.5 micron, d50 between 0.6 micron and 1 micron, and d90 between 2.4 microns and 3 microns, a particle-size distribution dX of Y denoting that X% of particles have a size less than Y. The powder may include or consist essentially of one or more metals (e.g., refractory metals such as tungsten). A super-atmospheric pressure is applied to the mold and/or the slip during and/or after introducing the slip into the mold. The mold may contain substantially only the slip.

These and other objects, along with advantages and features of the present invention herein disclosed, will become more apparent through reference to the following description, the accompanying drawings, and the claims. Furthermore, it is to be understood that the features of the various embodiments described herein are not mutually exclusive and may exist in various combinations and permutations. As used herein, the terms "approximately" and "substantially" mean ±10%, and in some embodiments, ±5%. The term "consists essentially of' means excluding other materials that contribute to function, unless otherwise defined herein. Nonetheless, such other materials may be present, collectively or individually, in trace amounts. As used herein, "consisting essentially of at least one metal" refers to a metal or a mixture of two or more metals but not compounds between a metal and a non-metallic element or chemical species such as oxygen or nitrogen (e.g., metal nitrides or metal oxides); such non-metallic elements or chemical species may be present, collectively or individually, in trace amounts, e.g., as impurities.

### Brief Description of the Drawings

In the drawings, like reference characters generally refer to the same parts throughout the different views. Also, the drawings are not necessarily to scale, emphasis instead generally being placed upon illustrating the principles of the invention. In the following description, various embodiments of the present invention are described with reference to the following drawings, in which:
Figure 1 is a schematic cross-section of a slip being introduced into a mold in accordance with various embodiments of the invention;
Figure 2 is a schematic cross-section of a green body within a mold in accordance with various embodiments of the invention;
Figure 3 is a schematic cross-section of an article after casting in accordance with various embodiments of the invention;
Figure 4 is a micrograph depicting the microstructure of a cast article in accordance with various embodiments of the invention; and
Figures 5A-5C are schematic cross-sections of fabrication of an article via pressure casting in accordance with various embodiments of the invention.

### Detailed Description

In order to enable slip and pressure casting without the need for added suspension aids, the metal powder utilized in accordance with embodiments of the present invention has a particle-size distribution (PSD) that maintains an advantageous ratio between the powder sedimentation rate and the viscosity of the slip. In various embodiments, the metal powder has a PSD d10 between 0.15 micron and 0.5 micron, e.g., 0.3 micron, a PSD d50 between 0.6 micron and 1 micron, e.g., 0.8 micron, and a PSD d90 between 2.4 microns and 3 microns, e.g., 2.7 microns. (As known to the skilled practitioner, a PSD d10 value of X indicates that 10% of the powder particles have a size less than X.) Powders having desired PSDs may be prepared via, for example, deagglomeration and blending of commercially available powders. In various embodiments, the slip has a viscosity 0.7 and 1.3 Pa-s, and preferably between 0.9 and 1.1 Pa-s. In contrast, use of powders having conventional PSDs without suspension aids typically results in high sedimentation rates and low viscosities (e.g., below 0.5 Pa-s) unsuitable for slip casting.

For example, in an embodiment, a tungsten powder having a small Fisher sub-sieve sizer (FSSS) particle size is identified. (As known to the skilled practitioner, FSSS particle size represents the average particle size as determined by air permeability, assuming perfectly spherical powder particles.) In an embodiment, the FSSS particle size of the starting powder is between 0.5 micron and 1 micron, e.g., 0.7 micron. For example, an initial powder may be HC70S tungsten powder having an FSSS particle size of 0.7 micron, available from H.C. Starck GmbH of Goslar, Germany. Such powder may have a PSD d10 of 0.42 micron, d50 of 1.8 micron, and d90 of 3.8 microns. All or a portion of the initial powder may be deagglomerated by, e.g., ball milling with tungsten carbide milling balls in order to reduce agglomeration of the powder or ultrasonification (i.e., application of ultrasound energy) for a time sufficient to reduce or substantially eliminate agglomeration of the powder.

In an embodiment, a powder blend may be subsequently produced by blending an unmilled portion of the initial powder with a portion that has been deagglomerated in order to form a powder having the desired particle-size distribution. An exemplary powder blend may include, e.g., between 60% and 80% (e.g., 70%) by weight unmilled powder and between 20% and 40% (e.g., 30%) by weight deagglomerated powder. In an embodiment utilizing HC70S tungsten powder as the initial powder, the resulting powder blend may have a PSD d10 of 0.3 micron, d50 of 0.8 micron, and d90 of 2.7 microns.

After the powder having the engineered particle-size distribution is produced, the powder is suspended in a liquid including or consisting essentially of water, e.g., DI water. The resulting slip preferably contains between 30% and 40% (e.g., approximately 35%) of the solid particles by volume. As shown in Figure 1, the slip 100 is poured into a porous mold 110, e.g., a mold including or consisting essentially of gypsum, resin, one or more polymeric materials (e.g., polystyrene), and/or plaster of paris, having the desired shape and dimensions for a pre-sintered part (i.e., the shape and dimensions that, after sintering, provide the part with substantially the final desired shape and dimensions). In various embodiments of the invention, external pressure is applied while filling the mold 110 with the slip 100, as described in more detail below. For example, the slip 100 may be pumped into the mold 110 at a pressure exceeding atmospheric pressure. The density of the cast slip 100 may be, for example, between 30% and 40%, e.g., approximately 34%, as determined by gravimetric methods. The liquid suspending the powder is then absorbed into mold 110, as shown in Figure 2, resulting in a green body 200 shaped by the mold 110. As shown in Figure 3, the green body 200 is removed from the mold 110 and subsequently sintered for densification, producing a sintered part 300. High-pressure air and/or vacuum may be applied via lines 530, 540 (either together or in sequence) in order to facilitate removal of the green body 200 from the mold 110. In an exemplary embodiment, the green body 200 is sintered in a hydrogen ambient. The sintering may be performed at temperatures between approximately 3000 °F (1649°C) and approximately 5000 °F (2760°C), e.g., approximately 4000 °F (2204°C), for a time period between approximately 2 hours and approximately 7 hours, e.g., approximately 5 hours.

After sintering, the part 300 may have a grain size smaller than approximately 30 microns, e.g., between approximately 10 microns and approximately 20 microns. The density of part 300 may be between approximately 95% and approximately 99% of its theoretical density, e.g., approximately 97%. The part may be utilized in its as-cast and as-sintered form, or may be machined into a desired shape, as, e.g., a crucible, a heat shield, a seamless tube, or other hollow or conical shape. Figure 4 is an optical micrograph of the microstructure of a part 300 fabricated from W powder in accordance with embodiments of the present invention. As shown in Figure 4, the grain size of the part 300 ranges between approximately 10 microns and approximately 20 microns. In Figure 4, the grains of part 300 have been revealed via etching with Murakami's etchant, known to those of skill in the art to be a mixture of potassium ferricyanide (K₃Fe(CN)₆), potassium hydroxide (KOH), and water.

Embodiments of the invention utilize pressure casting of powders having engineered PSDs to form metal parts. Figure 5A depicts a pressure casting apparatus 500 that may be utilized in embodiments of the present invention. As shown, apparatus 500 features a mold 110 partially or substantially encased within a pressure jacket 510 that may include or consist essentially of one or more mechanically strong and rigid materials capable of resisting the pressures imparted upon the slip while preventing deformation or fracture of the mold 110. As shown, the pressure jacket 510 (and the mold 110) may be composed of multiple different parts that may be separated (see Figure 5C) to facilitate removal of the cast part from the mold 110. Pressure jacket 510 of Figures 5A-5C is depicted as being composed of pressure-jacket portions 510-1, 510-2. The slip 100 is introduced into the mold 110 via a slip feed line 520 through which the slip 100 may be pumped under applied pressure. The apparatus 500 also includes pressure lines 530, 540 for the introduction of, e.g., high-pressure air (or other gas, e.g., inert gas), to apply pressure to the slip 100 during casting. For example air of a first super-atmospheric pressure (i.e., having a pressure greater than atmospheric pressure) may be introduced into pressure line 530 to apply pressure to the mold 110 and the slip 100, and either air of a second pressure less than the first super-atmospheric pressure or vacuum may be applied via the pressure line 540. The applied pressure may be substantially hydrostatic pressure, and it may advantageously decrease the amount of time required for the casting process (due to, e.g., increased outflow of water from the slip 100 during casting) and/or increase the density (and/or improve other mechanical properties) of the resulting green body. Pressures of greater than approximately 10 bars, greater than approximately 20 bars, or even greater than approximately 40 bars may be applied during casting in accordance with various embodiments of the present invention.

Figure 5B depicts apparatus 500 after the slip 100 has been introduced into the mold 110 via the slip feed line 520. After introduction of the slip 100, pressure is applied to the slip 100 within the mold 110 as detailed above in reference to Figure 5A, resulting in a green body 200 shaped by the mold 110. As shown in Figure 5C, the pressure jacket 510 and/or mold 110 may be separated into multiple portions to facilitate removal of the green body 200 from the mold 110. After pressure casting, the green body 200 may be sintered for densification, producing a sintered part 300. In an exemplary embodiment, the green body 200 is sintered in a hydrogen ambient. The sintering may be performed at temperatures between approximately 3000 °F (1649°C) and approximately 5000 °F (2760°C), e.g., approximately 4000 °F (2204°C), for a time period between approximately 2 hours and approximately 7 hours, e.g., approximately 5 hours.

The terms and expressions employed herein are used as terms and expressions of description and not of limitation, and there is no intention, in the use of such terms and expressions, of excluding any equivalents of the features shown and described or portions thereof. In addition, having described certain embodiments of the invention, it will be apparent to those of ordinary skill in the art that other embodiments incorporating the concepts disclosed herein may be used without departing from the scope of the invention, which is defined by the following claims. Accordingly, the described embodiments are to be considered in all respects as only illustrative and not restrictive.

## Claims

1. A method of producing a shaped part, the method comprising:
- suspending, in a liquid consisting of water, a powder comprising one or more refractory metals having a Fisher sub-sieve sizer (FSSS) particle-size distribution as determined by air permeability assuming perfectly spherical powder particles of d10 between 0.15 micron and 0.5 micron, d50 between 0.6 micron and 1 micron, and d90 between 2.4 microns and 3 microns, thereby forming a slip, wherein a particle-size distribution dX of Y denotes that X% of particles have a size less than Y;
- introducing the slip into a mold having a shape approximately equal to a desired shape of the shaped part, the particle-size distribution of the powder comprising one or more refractory metals (i) substantially preventing separation of the powder comprising one or more refractory metals from the liquid by at least one of agglomeration or sedimentation and (ii) maintaining a substantially homogeneous distribution of powder particles comprising one or more refractory metals within the liquid;
- thereafter, allowing at least a portion of the liquid to drain out of the slip to produce a green body comprising the powder comprising one or more refractory metals, further comprising applying a super-atmospheric pressure to at least one of the mold or the slip during or after introducing the slip into the mold; and
- sintering the green body to produce the shaped part.

2. The method of claim 1, wherein the particle-size distribution of the powder comprising one or more refractory metals is d10 of approximately 0.3 micron, d50 of approximately 0.8 micron, and d90 of approximately 2.7 microns, wherein the term "approximately" means ±10%.

3. The method of claim 1, wherein, after sintering, the shaped part has a density between 95% and 99% of theoretical density.

4. The method of claim 1, wherein, after sintering, the shaped part has a grain size between approximately 10 microns and approximately 20 microns, wherein the term "approximately" means ±10%.

5. The method of claim 1, wherein the powder comprising one or more refractory metals comprises at least one of tungsten, tantalum, niobium, zirconium, molybdenum, or titanium.

6. The method of claim 1, wherein the powder comprising one or more refractory metals comprises tungsten.

7. The method of claim 1, wherein the green body is sintered in hydrogen.

8. The method of claim 1, wherein the green body is sintered at a temperature between approximately 1649°C and approximately 2760°C, wherein the term "approximately" means ±10%.

9. The method of claim 1, further comprising producing the powder comprising one or more refractory metals by a process comprising:
- providing an initial powder comprising one or more refractory metals having a particle-size distribution d10 of approximately 0.42 micron, d50 of approximately 1.8 micron, and d90 of approximately 3.8 microns;
- deagglomerating a portion of the initial powder comprising one or more refractory metals, wherein the term "approximately" means ±10%; and
- blending the deagglomerated portion of the initial powder comprising one or more refractory metals with a second portion of the initial powder comprising one or more refractory metals, wherein preferably, the portion of the initial powder comprising one or more refractory metals is deagglomerated by ball milling.

10. The method of claim 1, wherein a density of the green body is between approximately 30% and approximately 40% of theoretical density, wherein the term "approximately" means ±10%.

11. The method of claim 1, wherein the liquid consists of deionized water.

12. The method of claim 1, wherein (i) the mold is porous and (ii) substantially all of the liquid from the slip drains into the mold to form the green body.

13. The method of claim 1, wherein neither the slip nor the mold is agitated after the slip is introduced into the mold.

14. The method of claim 1, wherein the powder comprising one or more refractory metals is substantially homogeneously distributed within the green body, or, further comprising machining the shaped part to a desired size and/or shape.

## Patentansprüche

1. Verfahren zur Herstellung eines Formteils, wobei das Verfahren umfasst:
- Suspendieren eines Pulvers in einer aus Wasser bestehenden Flüssigkeit, das ein oder mehrere hochschmelzende Metalle mit einem Fisher-Sub-Sieve-Sizer (FSSS) mit einer Teilchengrößenverteilung, wie sie durch Luftdurchlässigkeit bestimmt wird, wobei vollkommen kugelförmige Pulverteilchen von d10 zwischen 0,15 Mikrometer und 0,5 Mikrometer, d50 zwischen 0,6 Mikrometer und 1 Mikrometer und d90 zwischen 2,4 Mikrometer und 3 Mikrometer angenommen werden, wodurch ein Schlicker gebildet wird, wobei eine Teilchengrößenverteilung dX von Y bedeutet, dass X % der Teilchen eine Größe von weniger als Y aufweisen;
- Einführen des Schlickers in eine Form mit einer Gestalt, die etwa gleich einer gewünschten Gestalt des Formteils ist, wobei die Teilchengrößenverteilung des Pulvers ein oder mehrere hochschmelzende Metalle umfasst, (i) im Wesentlichen die Trennung des Pulvers, das ein oder mehrere hochschmelzende Metalle umfasst, von der Flüssigkeit durch mindestens eines von Agglomeration oder Sedimentation verhindert und (ii) eine im Wesentlichen homogene Verteilung der Pulverteilchen, die ein oder mehrere hochschmelzende Metalle umfassen, in der Flüssigkeit aufrechterhält;
- danach Ermöglichen, dass mindestens ein Anteil der Flüssigkeit aus dem Schlicker abfließt, um einen Grünkörper zu erzeugen, der das Pulver umfasst, das ein oder mehrere hochschmelzende Metalle umfasst, weiterhin umfassend das Anlegen eines überatmosphärischen Drucks an mindestens eine der Formen oder den Schlicker während oder nach dem Einführen des Schlickers in die Form; und
- Sintern des Grünkörpers zur Herstellung des Formteils.

2. Verfahren nach Anspruch 1, wobei die Teilchengrößenverteilung des Pulvers, das ein oder mehrere hochschmelzende Metalle umfasst, d10 von etwa 0,3 Mikrometer, d50 von etwa 0,8 Mikrometer und d90 von etwa 2,7 Mikrometer beträgt, wobei der Begriff "etwa" ±10 % bedeutet.

3. Verfahren nach Anspruch 1, wobei das Formteil nach dem Sintern eine Dichte zwischen 95 % und 99 % der theoretischen Dichte aufweist.

4. Verfahren nach Anspruch 1, wobei das Formteil nach dem Sintern eine Korngröße zwischen etwa 10 Mikrometer und etwa 20 Mikrometer aufweist, wobei der Begriff "etwa" ±10 % bedeutet.

5. Verfahren nach Anspruch 1, wobei das Pulver, das ein oder mehrere hochschmelzende Metalle umfasst, mindestens eines von Wolfram, Tantal, Niob, Zirkonium, Molybdän oder Titan umfasst.

6. Verfahren nach Anspruch 1, wobei das Pulver, das ein oder mehrere hochschmelzende Metalle umfasst, Wolfram umfasst.

7. Verfahren nach Anspruch 1, wobei der Grünkörper in Wasserstoff gesintert wird.

8. Verfahren nach Anspruch 1, wobei der Grünkörper bei einer Temperatur zwischen etwa 1649°C und etwa 2760°C gesintert wird, wobei der Begriff "etwa" ±10 % bedeutet.

9. Verfahren nach Anspruch 1, weiterhin umfassend die Herstellung des Pulvers, das ein oder mehrere hochschmelzende Metalle umfasst, durch ein Verfahren, umfassend:
- Bereitstellen eines Ausgangspulvers, das ein oder mehrere hochschmelzende Metalle mit einer Teilchengrößenverteilung d10 von etwa 0,42 Mikrometer, d50 von etwa 1,8 Mikrometer und d90 von etwa 3,8 Mikrometer umfasst;
- Deagglomerieren eines Anteils des Ausgangspulvers, das ein oder mehrere hochschmelzende Metalle umfasst, wobei der Begriff "etwa" ±10 % bedeutet; und
- Mischen des deagglomerierten Anteils des Ausgangspulvers, das ein oder mehrere hochschmelzende Metalle umfasst, mit einem zweiten Anteil des Ausgangspulvers, das ein oder mehrere hochschmelzende Metalle umfasst, wobei vorzugsweise der Anteil des Ausgangspulvers, der ein oder mehrere hochschmelzende Metalle umfasst, durch Kugelmahlen deagglomeriert wird.

10. Verfahren nach Anspruch 1, wobei eine Dichte des Grünkörpers zwischen etwa 30 % und etwa 40 % der theoretischen Dichte liegt, wobei der Begriff "etwa" ±10 % bedeutet.

11. Verfahren nach Anspruch 1, wobei die Flüssigkeit aus desionisiertem Wasser besteht.

12. Verfahren nach Anspruch 1, wobei (i) die Form porös ist und (ii) im Wesentlichen die gesamte Flüssigkeit aus dem Schlicker in die Form abläuft, um den Grünkörper zu bilden.

13. Verfahren nach Anspruch 1, wobei weder der Schlicker noch die Form nach dem Einbringen des Schlickers in die Form bewegt wird.

14. Verfahren nach Anspruch 1, wobei das Pulver, das ein oder mehrere hochschmelzende Metalle umfasst, im Wesentlichen homogen innerhalb des Grünkörpers verteilt ist, oder weiterhin umfassend die spanabhebende Bearbeitung des Formteils zu einer gewünschten Größe und/oder Gestalt.

## Revendications

1. Procédé de production d'une pièce façonnée, le procédé comprenant :
- mettre en suspension, dans un liquide constitué d'eau, une poudre comprenant un ou plusieurs métaux réfractaires ayant une répartition granulométrique Fisher Sub-Sieve Sizer (FSSS) telle que déterminée par perméabilité à l'air en supposant des particules de poudre parfaitement sphériques de d10 entre 0,15 micron et 0,5 micron, d50 entre 0,6 micron et 1 micron, et d90 entre 2,4 microns et 3 microns, en formant ainsi une barbotine, dans lequel une répartition granulométrique dX de Y indique que X % de particules ont une taille inférieure à Y ;
- introduire la barbotine dans un moule ayant une forme approximativement égale à une forme souhaitée de la pièce façonnée, la répartition granulométrique de la poudre comprenant un ou plusieurs métaux réfractaires (i) empêchant sensiblement une séparation de la poudre comprenant un ou plusieurs métaux réfractaires du liquide par au moins l'une d'une agglomération ou d'une sédimentation, et (ii) maintenant une répartition sensiblement homogène de particules de poudre comprenant un ou plusieurs métaux réfractaires à l'intérieur du liquide ;
- ensuite, permettre à au moins une portion du liquide de s'écouler hors de la barbotine pour produire une ébauche crue comprenant la poudre comprenant un ou plusieurs métaux réfractaires, comprenant en outre l'application d'une pression super-atmosphérique à au moins l'un du moule ou de la barbotine pendant ou après l'introduction de la barbotine dans le moule ; et
- fritter l'ébauche crue pour produire la pièce façonnée.

2. Procédé selon la revendication 1, dans lequel la répartition granulométrique de la poudre comprenant un ou plusieurs métaux réfractaires est d10 d'approximativement 0,3 micron, d50 d'approximativement 0,8 micron, et d90 d'approximativement 2,7 microns, dans lequel le terme "approximativement" signifie ± 10 %.

3. Procédé selon la revendication 1, dans lequel, après le frittage, la pièce façonnée a une densité entre 95 % et 99 % d'une densité théorique.

4. Procédé selon la revendication 1, dans lequel, après le frittage, la pièce façonnée a une granulométrie entre approximativement 10 microns et approximativement 20 microns, dans lequel le terme "approximativement" signifie ± 10 %.

5. Procédé selon la revendication 1, dans lequel la poudre comprenant un ou plusieurs métaux réfractaires comprend au moins l'un parmi le tungstène, le tantale, le niobium, le zirconium, le molybdène ou le titane.

6. Procédé selon la revendication 1, dans lequel la poudre comprenant un ou plusieurs métaux réfractaires comprend du tungstène.

7. Procédé selon la revendication 1, dans lequel l'ébauche crue est frittée dans l'hydrogène.

8. Procédé selon la revendication 1, dans lequel l'ébauche crue est frittée à une température entre approximativement 1649 °C et approximativement 2760 °C, dans lequel le terme "approximativement" signifie ± 10 %.

9. Procédé selon la revendication 1, comprenant en outre la production de la poudre comprenant un ou plusieurs métaux réfractaires par un processus comprenant :
- prévoir une poudre initiale comprenant un ou plusieurs métaux réfractaires ayant une répartition granulométrique d10 d'approximativement 0,42 micron, d50 d'approximativement 1,8 micron, et d90 d'approximativement 3,8 microns ;
- désagglomérer une portion de la poudre initiale comprenant un ou plusieurs métaux réfractaires, dans lequel le terme "approximativement" signifie ± 10 % ; et
- mélanger la portion désagglomérée de la poudre initiale comprenant un ou plusieurs métaux réfractaires avec une seconde portion de la poudre initiale comprenant un ou plusieurs métaux réfractaires, dans lequel de préférence la portion de la poudre initiale comprenant un ou plusieurs métaux réfractaires est désagglomérée par broyage à boulets.

10. Procédé selon la revendication 1, dans lequel une densité de l'ébauche crue est entre approximativement 30 % et approximativement 40 % d'une densité théorique, dans lequel le terme "approximativement" signifie ± 10 %.

11. Procédé selon la revendication 1, dans lequel le liquide est constitué d'eau désionisée.

12. Procédé selon la revendication 1, dans lequel (i) le moule est poreux et (ii) sensiblement l'intégralité du liquide de la barbotine s'écoule dans le moule pour former l'ébauche crue.

13. Procédé selon la revendication 1, dans lequel ni la barbotine ni le moule ne sont agités après l'introduction de la barbotine dans le moule.

14. Procédé selon la revendication 1, dans lequel la poudre comprenant un ou plusieurs métaux réfractaires est répartie de manière sensiblement homogène à l'intérieur de l'ébauche crue, ou, comprenant en outre l'usinage de la pièce façonnée à une taille et/ou à une forme souhaitée.
